# EUROPEAN PATENT APPLICATION

(11) **EP 0 583 834 A1**
(43) Date of publication of application: **23.02.1994**
(21) Application number: 93202387.2
(22) Date of filing: 14.08.1993
(51) Int. Cl.: G03C 7/327

(54) **Color photographic materials containing 5-pyrazolone polymeric couplers**

(30) Priority: 19.08.1992 US 932409
(71) Applicant: EASTMAN KODAK COMPANY, Rochester, New York 14650-2201 (US)
(72) Inventor: Schofield, Edward, c/o EASTMAN KODAK COMPANY, Rochester, New York 14650-2201 (US); Chen, Tien-Teh, c/o EASTMAN KODAK COMPANY, Rochester, New York 14650-2201 (US); Youngblood, Michael P., c/o EASTMAN KODAK COMPANY, Rochester, New York 14650-2201 (US)
(74) Representative: Baron, Paul Alexander Clifford

(57) **Abstract**

Color photographic materials comprise a supporting substrate having coated thereon a silver halide emulsion and a polymeric coupler having repeating units of the formula (I):
wherein Q represents a coupler group derived from a 5-pyrazolone.

## Description

### FIELD OF THE INVENTION

The present invention relates to color photographic materials containing 5-pyrazolone polymeric couplers. More specifically, the present invention relates to color photographic materials containing 5-pyrazolone polymeric couplers formed from at least one dye-forming monomer and at least one non-dye-forming monomer.

### BACKGROUND OF THE INVENTION

Color photographic materials containing a silver halide emulsion are well known in the art, as is the development of such materials involving the reaction of an oxidized aromatic primary amine color developing agent with a dye-forming coupler. Various yellow, cyan and magenta dye-forming couplers are also known in the art. Particularly, the Ichijima et al U.S. Patents Nos. 4,301,235 and 4,310,619 and the Hirose et al U.S. Patent No. 4,584,226 disclose 2-equivalent 5-pyrazolone magenta dye-forming couplers for use in silver halide color photographic materials.

It is also known in the art that couplers may be incorporated in the form of a polymer which improves the ability of the dye to remain in the location where it is formed in a color photographic element. For example, Monbaliu et al. disclose (U.S. Patent No. 3,926,436) photographic elements containing polymeric couplers as latexes which show less foaming tendency and which show high compatibility with hydrophilic colloids such as gelatin. Yagihara et al. (U.S. Patent No. 4,474,870) disclose photographic materials containing polymeric coupler latexes that form magenta dyes upon coupling with oxidized developing agents. Hirano et al (U.S. Patent No. 4,511,647) disclose color photographic materials containing cyan color forming coupler latexes. Yagihara et al. (U.K. Patent No. 2,092,573 B) disclose silver halide photographic materials containing magenta color forming coupler latexes. Cawse and Harris (European Patent Application 0321399 A3) disclose a method of preparing latexes of color couplers.

Generally, three methods have been employed in the past for dispersing polymeric couplers. These three methods include: (1) dispersing the coupler by colloid milling or homogenization methods, along with high and/or low vapor pressure organic solvents in aqueous surfactant and gelatin; (2) direct incorporation of solutions of water soluble polymers; (3) latex formation by emulsion polymerization or suspension polymerization.

Hirano (U.S. Patent No. 4,522,916) discloses the preparation of polymeric magenta dye forming coupler latexes that provide images of improved light stability. Hirano and Furutachi (U.S. Patent No. 4,576,910) disclose the preparation of polymeric magenta dye forming coupler latexes formed from triazole and tetrazole monomers. Helling et al. (U.S. Patent No. 4,756,998) disclose the preparation of polymeric couplers which contain at least one urethane or urea group. Yamanouchi et al. (U.S. Patent No. 4,874,689) disclose the preparation of polymeric couplers utilizing chain transfer agents of eight or more carbon atoms. Helling (U.S. Patent No. 4,921,782) discloses the preparation of polymeric magenta dye forming couplers, wherein the magenta coupler monomer contains a carboxyl group. Maekawa and Hirano (U.S. Patent No. 4,946,771) disclose the preparation of polymeric couplers formulated with certain advantageously incorporated coupling and noncoupling comonomers.

Polymeric couplers can be prepared by joining reactive couplers to synthesized polymers. Such polymers may include polyacrylic acid, poly-p-aminostyrene, and other natural high polymers. Methods for producing such polymeric couplers are described in U.S. Patents Nos. 2,698,797, 2,852,381, 2,852,383 and 2,870,712 and in Japanese Patent Publications Nos. 16932/1960 and 3661/1969. Methods for forming polymeric couplers from ethylenically unsaturated monomers and other polymerizable monomers are disclosed in British Patents Nos. 880,206, 955,197, 967,503, 967,504, 995,363, and 1,104,658.

Jones discloses (U.S. Patent No. 2,561,205) the formation of water-soluble polymeric couplers derived from beta, gamma-ethylenically unsaturated amides. Williams discloses (U.S. Patent No. 2,739,956) the formation of water-soluble polymeric couplers derived from vinyl-substituted monomers such as 2-vinyl-l-naphthol. Firestine discloses (U.S. Patent No. 2,976,294) water-soluble polymers derived from methacrylamide related monomers, such as 1-(m-methacryloylaminophenyl)-2-carboxy-5-pyrazolone.

Umberger (U.S. Patent No. 3,451,820) discloses dispersions of lipophilic color-forming polymeric couplers. Van Paesschen and Priem (U.S. Patent No. 4,080,211) disclose a process for making color-coupling agents by emulsion polymerization. Ponticello et al. (U.S. Patent No. 4,215,195) disclose the preparation of cross-linkable polymers that contain color-forming coupler residues. Hirano et al. (U.S. Patent No. 4,518,687) disclose a photographic material containing a cyan dye-forming oleophilic polymeric coupler. Lau and Tang (U.S. Patent No. 4,612,278) disclose photographic materials containing polymeric couplers copolymerized with alkoxyalkylacrylate monomers.

Retouching of color photographic images is well known in the art, especially in the reversal film system. Retouching is carried out after the photographic material has been developed and processed. During retouching, magenta, yellow or cyan image dye may be selectively removed using appropriate bleach solutions. The ability to selectively bleach a color photographic image dye is an important characteristic of the parent image coupler.

### SUMMARY OF THE INVENTION

It is therefore an object of the present invention to provide color photographic materials comprising a silver halide emulsion and a polymeric coupler. It is a further object of the invention to provide such color photographic materials having one or more improved properties useful in forming color images. It is a more specific object of the invention to provide color photographic materials comprising a silver halide emulsion and a polymeric coupler which forms an image dye that can be selectively bleached during retouching of the photographic material.

These and additional objects are provided by the color photographic materials of the present invention which comprise a supporting substrate having coated thereon a silver halide emulsion and a polymeric coupler. The polymeric coupler comprises repeating units according to the formula (I)
wherein R¹ and R² are, independently, hydrogen or methyl;
R³ is hydrogen, methyl or ethyl;
D represents at least one additional polymerized monomer;
x is from about 20 to 80 mole percent;
y is from about 20 to 80 mole percent;
z is from 0 to about 50 mole percent;
A is a -CONH-, -COO-, -O- or phenylene group;
B is an unsubstituted or substituted, straight or branched alkylene group, an unsubstituted or substituted, straight or branched aralkylene group, or a unsubstituted or substituted phenylene group;
Y is -(O(CH2)m)n-, -OCOO-, -OCONH-, -CONR'-, -NR'CONR'-, -NR'COO-, -NR'CO-, -OCONR'-, -NR'-, -COO-, -OCO-, -CO-, -O-, -SO₂-, -NR'SO₂-, and -SO₂NR'-, wherein m is from 1 to 4, n is from 1 to 8, and R' is a hydrogen atom, or a substituted or unsubstituted alkyl group, or a substituted or unsubstituted aryl group, and when two or more R' substituents are present in Y, the two or more R' substituents may be the same or different;
q is 0 or 1;
p is the same as q;
r is from 1 to 8;
Q represents a coupler group derived from a 5-pyrazolone; and
E is -O- or -NH-.

The present Inventors have discovered that the magenta image dye formed from the pyrazolone-containing polymeric couplers included in the present color photographic materials can be selectively bleached, for example, using an aqueous stannous chloride solution, whereby the photographic materials of the present invention are particularly suitable for use in reversal film systems.

These and additional objects and advantages provided by the color photographic materials of the present invention will be more fully apparent in view of the following detailed description.

### DETAILED DESCRIPTION

The color photographic materials of the present invention comprise a supporting substrate having coated thereon a silver halide emulsion and a magenta dye-forming 5-pyrazolone polymeric coupler.

The 5-pyrazolone coupler groups are well known in the art as demonstrated, for example, in the Ichijima et al U.S. Patents Nos. 4,301,235 and 4,310,619. In a preferred embodiment of the polymeric coupler, Q is selected from the formulas (II)-(IV):
wherein * represents the site for linkage to (Y)_{q};
R⁴ is arylamino, carbonamido, ureido, sulfonamido, alkylamino, or a heterocyclic amino group, all of which groups may be substituted or unsubstituted;
R⁵ is a substituted or unsubstituted alkyl group or a substituted or unsubstituted aryl group;
X is hydrogen or a group capable of being released by a coupling reaction with an oxidized aromatic primary amine developing agent; and
X' is a divalent group derived from X having bonding sites to the pyrazolone ring and to (Y)_{q}. In a preferred embodiment, R5 in the coupler group Q comprises a substituted or unsubstituted aryl group. Suitable substituents for the aryl group include, but are not limited to, halogen atoms and cyano, alkylsulfonyl, arylsulfonyl, sulfamoyl, sulfonamido, carbamoyl, carbonamido, alkoxy, acyloxy, aryloxy, alkoxycarbonyl, aryloxycarbonyl, ureido, nitro, alkyl and trifluromethyl groups. Halogen-substituted aryl groups are particularly preferred.

In a further preferred embodiment, the coupler group Q is of formula (II), in which R5 is selected from the group consisting of substituted and unsubstituted aryl groups, and X represents:
wherein Zₐ, Z_{b}, Z_{c}, and Z_{d} are independently selected from the group consisting of substituted or unsubstituted methine groups and -N=. Suitable substituents for the methine group include, but are not limited to, substituted and unsubstituted alkyl groups and substituted and unsubstituted aryl groups. Examples of the nitrogen containing heterocyclic groups formed by Zₐ, Z_{b}, Z_{c} and Z_{d} and the tertiary nitrogen atom include a pyrazolyl group, an imidazolyl group, a triazolyl group, a tetrazolyl group, and the like. Of these, a pyrazolyl group in which Za represents -N= and Z_{b}, Z_{c} and Z_{d} each represents a methine group or a substituted methine group is particularly preferred. In a further preferred embodiment, all of Z_{b}, Z_{c} and Z_{d} are unsubstituted.

With further reference to the polymeric coupler repeating units of formula (I), in a preferred embodiment, A is -CONH-, and p and q are 0. In a further preferred embodiment, r is 1 and R³ is an ethyl or methyl group. Moreover, while x may range from about 20 to 80 mol percent, y may range from 20 to 80 mol percent and z may be up to about 50 mol percent, in a further preferred embodiment, x is from about 30 to 60 mol percent, y is from about 30 to 60 mol percent and z is from 0 to about 25 mol percent. When z is greater than 0 and the at least one additional polymerized monomer D is present in the polymeric coupler, the repeating unit D may be formed from any suitable ethylenically unsaturated monomer. Suitable examples of the ethylenically unsaturated monomer from which the repeating unit D is polymerized include, but are not limited to, esters, for example, lower alkyl esters such as methyl acrylate, ethyl acrylate, propyl acrylate, butyl acrylate, ethylhexyl acrylate, hexyl acrylate, methyl methacrylate, octyl methacrylate, lauryl methacrylate, vinyl esters such as vinyl acetate, vinyl propionate, vinyl laurate, acrylonitrile, methacrylonitrile, amides, for example, acrylamide and methacrylamide, vinyl aromatics, for example, styrene and derivatives thereof including vinyl toluene, divinylbenzene, vinyl ethers, and the like. In one embodiment, D is the same as the previous repeating unit in Formula (I), i.e. the repeating unit containing the variables R², E and R³, except that the R3 in the D repeating unit is different from the R³ in the previous repeating unit in Formula (I).

The polymeric couplers according to the present invention may be formed by any of the known polymerization techniques for the polymerization of ethylenically unsaturated monomers. Emulsion polymerization methods are particularly suitable as disclosed in the Yagihara et al U.S. Patent No. 4,367,282. In accordance with well known polymerization techniques, the polymeric couplers may be formed as homogeneous latex particles or, alternatively, may be in the form of core-shell latex particles as taught, for example, in the Hirano et al U.S. Patent No. 4,444,870.

Alternatively, the polymer latex is formed by solution polymerization of monomer mixture comprising a coupler monomer, a comonomer, and an ionic comonomer containing sulfonic, sulfuric, sulfinic, carboxylic or phosphoric acid, such as acrylamido-2,2'-dimethyl-propane sulfonic acid, 2-sulfoethyl methacrylate, or sodium styrene sulfonate. The polymer solution obtained is then dispersed in aqueous solution to form a latex.

A third way of forming polymer latex is by solution polymerization of monomer mixture comprising a coupler monomer and comonomers. An organic solvent is used for dissolving the polymeric coupler and the solution is dispersed in an aqueous solution of gelatin in the form of latex as described in U.S. Patents Nos. 4,668,613; 4,874,689 and 4,946,771.

Specific polymeric couplers for use in the color photographic materials of the present invention, include, but are not limited to, couplers comprising repeating units according to the following formulas:

The photographic materials of the present invention may be simple elements or multilayer, multicolor elements. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art.

A typical multicolor photographic element comprises a support bearing a cyan dye image-forming unit comprising at least one red-sensitive silver halide emulsion layer having associated therewith at least one cyan dye-forming coupler, a magenta image-forming unit comprising at least one green-sensitive silver halide emulsion layer having associated therewith at least one magenta dye-forming coupler and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers, and the like. The element typically will have a total thickness (excluding the support) of from 5 to 30 microns. The support may be transparent or reflective.

Suitable materials for use in the elements of this invention are disclosed in Research Disclosure, December 1978, Item 17643; January 1983, Item 22534; and December 1989, Item No. 308119 published by Kenneth Mason Publications, Ltd., Dudley Annex, 12a North Street, Emsworth, Hampshire P010 7DQ, ENGLAND. This publication will be identified hereafter by the term "Research Disclosure." The elements of the invention can comprise emulsions and addenda described in these publications and publications referenced in these publications.

The silver halide emulsions employed in the color photographic materials of this invention can be comprised of silver bromide, silver chloride, silver iodide, silver chlorobromide, silver chloroiodide, silver bromoiodide, silver chlorobromoidide or mixtures thereof. The emulsions can include silver halide grains of any conventional shape or size. Specifically, the emulsions can include coarse, medium or fine silver halide grains. Useful tabular grain emulsions are described in Research Disclosure, Item 22534, and in U.S. Patent No. 4,748,106. High aspect ratio tabular grain emulsions are specifically contemplated, such as those disclosed by Wilgus et al U.S. Patent 4,434,226, Daubendiek et al U.S. Patent 4,424,310, Wey U.S. Patent 4,399,215, Solberg et al U.S. Patent 4,433,048, Mignot U.S. Patent 4,386,145, Evans et al U.S. Patent 4,504,570, Maskasky U.S. Patent 4,400,463, Wey et al U.S. Patent 4,414,306, Maskasky U.S. Patents 4,435,501 and 4,4414,966 and Daubendiek et al U.S. Patents 4,672,027 and 4,693,964. Also specifically contemplated are those silver bromoiodide grains with a higher molar proportion of iodide in the core of the grain than in the periphery of the grain, such as those described in British Reference No. 1,027,146; Japanese Reference No. 54/48,521; U.S. Patents Nos. 4,379,837; 4,444,877; 4,665,012; 4,686,178; 4,565,778; 4,728,602; 4,668,614 and 4,636,461; and in European Reference No. 264,954. The silver halide emulsions can be either monodisperse or polydisperse as precipitated. The grain size distribution of the emulsions can be controlled by silver halide grain separation techniques or by blending silver halide emulsions of differing grain sizes.

Sensitizing compounds, such as compounds of copper, thallium, lead, bismuth, cadmium and Group VIII noble metals, can be present during precipitation of the silver halide emulsion.

The silver halide emulsions can be surface sensitized, and noble metal (e.g., gold), middle chalcogen (e.g., sulfur, selenium, or tellurium) and reduction sensitizers, employed individually or in combination, are specifically contemplated. Typical chemical sensitizers are listed in Research Disclosure, Item 17643, cited above, Section III.

Spectral sensitization of the silver halide emulsions by sensitizing dyes is disclosed, for example, in Research Disclosure, Item 17643, cited above, Section IV.

Suitable vehicles for the emulsion layers and other layers of elements of this invention are described in Research Disclosure Item 17643, Section IX and the publications cited therein.

In addition to the polymeric 5-pyrazolone magenta couplers described herein, the elements of this invention can include additional couplers as described in Research Disclosure Section VII, paragraphs D, E, F and G and the publications cited therein.

The photographic elements of this invention can contain brighteners (Research Disclosure Section V), antifoggants and stabilizers (Research Disclosure Section VI), antistain agents and image dye stabilizers (Research Disclosure Section VII, paragraphs I and J), light absorbing and scattering materials (Research Disclosure Section VIII), hardeners (Research Disclosure X), coating aids (Research Disclosure Section XI), plasticizers and lubricants (Research Disclosure Section XII), antistatic agents (Research Disclosure Section XIII), matting agents (Research Disclosure Sections XII and XVI) and development modifiers (Research Disclosure Section XXI).

The photographic elements can be coated on a variety of supports as described in Research Disclosure Section XVII and the references described therein.

The photographic elements of the invention can be exposed to actinic radiation, typically in the visible region of the spectrum, to form a latent image as described in Research Disclosure Section XVIII, and then processed to form a visible dye image as described in Research Disclosure Section XIX. Preferred color developing agents are p-phenylenediamines. Especially preferred are 4-amino-3-methyl-N,N-diethylaniline hydrochloride, 4-amino-3-methyl-N-ethyl-N-β-(methanesulfonamido)-ethylaniline sulfate hydrate, 4-amino-3-methyl-N-ethyl-N-β-hydroxyethylaniline sulfate, 4-amino-3-β-(methanesulfonamido)ethyl-N,N-diethylaniline hydrochloride and 4-amino-N-ethyl-N,N-diethylaniline hydrochloride and 4-amino-N-ethyl-N-(2-methoxyethyl)-m-toluidine di-p-toluenesulfonic acid.

As is known in the art, the solution used to selectively bleach magenta dyes typically comprises aqueous stannous chloride. The present Inventors have discovered that the 5-pyrazolone polymeric couplers of the present invention exhibit good selective bleachability. This feature is particularly important in reversal film systems whereby the color photographic materials of the present invention are particularly suitable for use in such reversal film systems.

The advantages of the color photographic materials of the present invention are demonstrated in the following example. Throughout the example and the entire specification, parts and percentages are by weight unless otherwise specified.

### EXAMPLE

In this example, color photographic materials containing polymeric couplers according to the present invention were tested for bleachability. For comparison purposes, color photographic materials containing nonpolymeric couplers and other polymeric couplers were also tested for bleachability.

The couplers were prepared as described in the following Synthesis Examples.
1. Synthesis of polymer P-1
   80g of deionized water and 4.4g of 10% sodium N-methyl-N-oleoyltaurate (Igepon T-77) were mixed in a 500mL 4-neck round bottom flask equipped with a mechanical stirrer, nitrogen inlet, and condenser. The flask was immersed into a constant temperature bath at 80oC and heated for 30 minutes with nitrogen purging through. 0.5g of methoxyethyl acrylate and 1 ml of 5% ammonium persulfate were added to the flask and polymerized for one hour. 1.3ml of 5% ammonium persulfate was further added. The monomer solution comprising 4.0g of N-(4',5'-dihydro-5'-oxo-1'-(2,4,6-trichlorophenyl)(1,4'-bi-1H-pyrazol)-3'-y1)-2-methyl-2-propenamide, 5.5g of methoxyethyl acrylate and 40 mL of ethanol was then added to the reactor over 3 hours and polymerized for 3 more hours. The latex was cooled, filtered and dialyzed against distilled water for overnight. It was then concentrated to 4.17% solid with Amicon's Ultrafiltration unit. The Z-average particle size measured by Malvern's Autosizer IIC was 120nm. The elemental analysis result was C(52%), H(5.9%), N(6.92%) and C1(11.00%). Yield was 80%.
2. Synthesis of polymer P-2
   440g of deionized water, 1.5g of sodium N-methyl-N-oleoyltaurate (Igepon T-77), and 40ml methanol were mixed in a 1L 4-neck round bottom flask equipped with a mechanical stirrer, nitrogen inlet, and condenser. The flask was immersed into a constant temperature bath at 80oC and heated for 30 minutes with nitrogen purging through. 6 ml of 5% ammonium persulfate was added and stirred for 3 minutes. The monomer solution comprising 12g of N-(4',5'-dihydro-5'-oxo-1'-(2,4,6-trichlorophenyl)(1,4'-bi-1H-pyrazol)-3'-y1)-2-methyl-2-propenamide, 18g of ethoxyethyl acrylate and 180mL of methanol was then added to the reactor over 3 hours and polymerized for 3 more hours. The latex was cooled, filtered and dialyzed against distilled water for overnight. It was then concentrated to 12.63% solid with Amicon's Ultrafiltration unit. The Z-average particle size measured by Malvern's Autosizer IIC was 65.8nm. The elemental analysis result was C(51.8%), H(6.0%), N(6.73%) and C1(1.29%). Yield was 77%.
   Polymers P-3 to P-12 and the Comparison polymers C-1 to C-18 and C-20 to C-22 set forth below were prepared by a similar method.
3. Synthesis of Comparison polymer C-19
   6.5g of pyrazotriazole coupler monomer, 1.75g of ethoxyethyl acrylate, 1.25g of acrylic acid, 0.5g of 2-acrylamido-2-methylpropane sulfonic acid, and 100ml of ethanol were mixed in a 250ml 3-neck flask equipped with condenser, nitrogen inlet, and magnetic stirrer. The solution was immersed in an oil bath and heated to 85°C until all the monomers were dissolved. 0.25g of azo-bis-isobutyronitrile (AIBN) in 5ml of ethanol was added to the flask. Polymerization was continued for 5 hours and 0.25g of AIBN was post added. The polymer solution was diluted with 50 ml ethanol and added to the 300 ml of hot distilled water with vigorous stirring. The thus formed polymer latex had a particle size of 60nm. Final % solid after Ultrafiltration was 5.6%. The Elemental analysis results were C(61%), H(7.6%), N(8.94%), and C1(4.5%). Yield was 82%.

The Comparison Couplers were of the following formulas:

In preparing the color photographic materials, gelatin, water, surfactant and TAI were combined and the respective coupler was added to the resulting solution. The polymeric couplers were added in the form of a polymer latex. The coupler-silver halide emulsion mixture was then coated on a supporting substrate. The exposure step was conducted for 0.02 sec and employed a 1B sensitometer, a 0-3 step tablet, a 0.9 neutral density filter and a DLV filter. The processing steps were conducted at 98.4°F as follows:

| **Step** | **Time** | **Atmosphere** |
|---|---|---|
| MQ Development | 6 minutes | N2 burst |
| Wash | 2 minutes | N2 burst |
| Reversal Bath | 2 minutes | N2 burst |
| Color Development | 6 minutes | N2 burst |
| Conditioner | 2 minutes | N2 burst |
| Bleach | (Table I) | Continuous Air |
| Fix | 4 minutes | Continuous Air |
| Wash | 4 minutes | Continuous Air |

In determining the bleachability, the following procedure was employed. The status A density (1.0) was read on a processed strip. A square (1/4 inch) was then blanked off on the processed strip using tape as a border. A swab was dipped in a fresh bleach solution and smeared on the squared portion for 6 minutes, after which the strip was washed in water for five minutes. After drying the status A density of the squared portion of film was reread and the percent of density loss was calculated.

Two types of bleaching solution were used. Bleach solution A comprised 5g stannous chloride (SnCl₂), 30 ml of a 10% H₂SO₄ solution and 65 ml water. Bleach solution B comprised 5g stannous chloride (SnCl₂), 30 ml of a 5% H₂SO₄ solution and 65 ml water.

To demonstrate the effect of the comonomers of the bleachability of the polymeric couplers, a series of polymeric 5-pyrazolone couplers with various types of comonomers were prepared. Three separate bleaching experiments were carried out and the results are shown in Table I - Table III.

**Table I**

| **Remark** | **Coupler No.** | **Bleaching Solution** | **% Loss** |
|---|---|---|---|
| Comparative | C-1 | A | 25.9 |
| Comparative | C-2 | A | 32.7 |
| Comparative | C-3 | A | 16.7 |
| Comparative | C-4 | A | 23.4 |
| Invention | P-1 | A | 48.9 |
| Invention | P-2 | A | 63.9 |
| Invention | P-3 | A | 79.8 |
| Invention | P-4 | A | 72.6 |

**Table II**

| **Remark** | **Coupler No.** | **Bleaching Solution** | **% Loss** |
|---|---|---|---|
| Comparative | C-5 | B | 24.3 |
| Comparative | C-6 | B | 3.7 |
| Comparative | C-7 | B | 16 |
| Comparative | C-8 | B | 0 |
| Comparative | C-9 | B | 15.4 |
| Invention | P-2 | B | 47.3 |
| Invention | P-1 | B | 45 |

**Table III**

| **Remark** | **Coupler No.** | **Bleaching Solution** | **% Loss** |
|---|---|---|---|
| Comparative | C-10 | B | 14.8 |
| Comparative | C-11 | B | 11.1 |
| Comparative | C-12 | B | 11.3 |
| Comparative | C-13 | B | 9.7 |
| Comparative | C-14 | B | 18 |
| Comparative | C-15 | B | 4.2 |
| Invention | P-5 | B | 42.5 |
| Invention | P-6 | B | 41 |
| Invention | P-7 | B | 49.4 |

It is clear from these results that polymeric 2 or 4 equivalent 5-pyrazolone couplers containing the comonomers of this invention exhibited significantly improved bleachability as compared with the comparison examples.

The 5-pyrazolone coupler moiety defined in this invention is essential for the selective bleaching. As set forth in Table IV, comparisons were made between polymeric couplers derived from 5-pyrazolone couplers and other magenta couplers, especially pyrazotriazole type magenta couplers. It is clear from Table IV that polymeric 5-pyrazolone couplers of this invention have much higher bleachability than the comparative polymeric and nonpolymeric magenta couplers.

**Table IV**

| **Remark** | **Coupler No.** | **Bleaching Solution** | **% Loss** |
|---|---|---|---|
| Comparative | C-16 | A | 0.3 |
| Comparative | C-17 | A | 1 |
| Comparative | C-18 | A | 0.5 |
| Comparative | C-19 | A | 0.8 |
| Comparative | C-20 | A | 0.7 |
| Comparative | C-21 | A | 1 |
| Invention | P-1 | A | 48.9 |
| Invention | P-2 | A | 63.9 |
| Invention | P-3 | A | 79.8 |
| Invention | P-4 | A | 72.6 |

The results set forth in Tables I-IV demonstrate that the polymeric couplers of this invention exhibit significantly improved bleachability. Thus, the color photographic materials of the present invention are particularly useful for reversal film systems.

## Claims

1. A color photographic material comprising a supporting substrate having coated thereon a silver halide emulsion and a polymeric coupler comprising repeating units according to formula (I): wherein R¹ and R² are, independently, hydrogen or methyl;
R³ is hydrogen, methyl or ethyl;
D represents at least one additional polymerized monomer;
x is from about 20 to 80 mole percent;
y is from about 20 to 80 mole percent;
z is from 0 to about 50 mole percent;
A is a -CONH-, -COO-, -O- or phenylene group;
B is an unsubstituted or substituted, straight or branched alkylene group, an unsubstituted or substituted, straight or branched aralkylene group, or an unsubstituted or substituted phenylene group;
Y is -(O(CH2)m)n-, -OCOO-, -OCONH-, -CONR'-, -NR'CONR'-, -NR'COO-, -NR'CO-, -OCONR'-, -NR'-, -COO-, -OCO-, -CO-, -O-, -SO₂-, -NR'SO₂-, and -SO₂NR'-, wherein m is from 1 to 4, n is from 1 to 8, and R' is a hydrogen atom, or a substituted or unsubstituted alkyl group, or a substituted or unsubstituted aryl group, and when two or more R' substituents are present in Y, the two or more R' substituents may be the same or different;
q is 0 or 1;
p is the same as q;
r is from 1 to 8;
Q represents a coupler group derived from a 5-pyrazolone; and
E is -O- or -NH-.

2. A color photographic material as defined by claim 1, wherein A is -CONH- and p and q are 0.

3. A color photographic material as defined in claim 1 or 2, wherein r is 1 and R³ is ethyl.

4. A color photographic material as defined in any of claims 1-3, wherein z is greater than 0, and D is formed from at least one ethylenically unsaturated monomer selected from acrylates, methacrylates, vinyl esters, acrylamides, methacrylamides, acrylonitrile, methacrylonitrile, vinyl ethers and vinyl aromatics.

5. A color photographic material as defined in any of claims 1-4 in which:x is from about 30 to 60 mole percent;
y is from about 30 to 60 mole percent; and
z is from 0 to about 25 mole percent.

6. A color photographic material according to any of claims 1-5 wherein Q has one of the formulas (II)-(IV): wherein * represents the site for linkage to (Y)_{q};
R⁴ is arylamino, carbonamido, ureido, sulfonamido, alkylamino, or a heterocyclic amino group, all of which groups may be substituted or unsubstituted;
R⁵ is a substituted or unsubstituted alkyl group or a substituted or unsubstituted aryl groups;
X is hydrogen or a group capable of being released by a coupling reaction with an oxidized aromatic primary amine developing agent; and
X' is a divalent group derived from X having bonding sites to the pyrazolone ring and to (Y)_{q}.

7. A color photographic material according to claim 6 wherein Q is of formula (II)wherein R⁵ is aa substituted or unsubstituted aryl group, and
X represents: wherein Zₐ, Z_{b}, Z_{c}, and Z_{d} are, independently, a substituted or unsubstituted methine group or -N=.

8. A color photographic material as defined by claim 7, wherein Zₐ is -N=.

9. A color photographic material as defined by claim 7 or 8, wherein Z_{b}, Z_{c} and Z_{d} are all unsubstituted methine groups.

10. A color photographic material as defined any of claims 7-9, wherein R⁵ is a halogen-substituted aryl group.
